# EUROPEAN PATENT SPECIFICATION

(11) **EP 3 318 667 B1**
(45) Date of publication and mention of the grant of the patent: **06.05.2020**
(21) Application number: 16818032.1
(22) Date of filing: 30.06.2016
(51) Int. Cl.: D04H 3/16, D01D 5/08, D04H 3/009, D01D 5/084, D01D 5/098, D01F 6/74, D01F 6/64

(54) **NONWOVEN FABRIC AND PRODUCTION METHOD FOR SAME**
VLIESSTOFF UND HERSTELLUNGSVERFAHREN DAFÜR
TISSU NON TISSÉ ET SON PROCÉDÉ DE PRODUCTION

(30) Priority: 30.06.2015 JP 2015131693
(43) Date of publication of application: 09.05.2018
(73) Proprietor: Kuraray Co., Ltd., Kurashiki-shi, Okayama 710-0801 (JP)
(72) Inventor: SHIRAISHI, Ikuhisa, Saijo-shi Ehime 793-8585 (JP); SHIROTANI, Yasuhiro, Saijo-shi Ehime 793-8585 (JP)
(74) Representative: Vossius & Partner Patentanwälte Rechtsanwälte mbB
(86) International application number: PCT/JP2016/069462
(87) International publication number: WO 2017/002924

(56) References cited:
- WO-A1-02/059403
- WO-A1-2015/080913
- JP-A- H0 860 515
- JP-A- H05 279 947
- JP-A- S63 315 655
- JP-A- 2004 185 860
- JP-A- 2008 081 893
- JP-A- 2012 041 644
- US-A1- 2011 076 907

## Description

### TECHNICAL FIELD

The present invention relates to a nonwoven fabric, and a method for producing the nonwoven fabric.

### BACKGROUND ART

In recent years, a nonwoven fabric made of ultra-fine fibers produced by a melt blown method or the like has been developed, and is used for various applications. With respect to a nonwoven fabric containing a polymer having a glass transition temperature (Tg) of less than 50°C, such as polypropylene and polyethylene, a nonwoven fabric excellent in the handleability, in which fibers are fused to one another, can be obtained without performing a post processing such as emboss processing, calender processing, or spunlace processing.

However, with respect to a nonwoven fabric containing a polymer that has a Tg of greater than or equal to 50°C, unless the fibers are fused to one another or three-dimensionally entangled with one another by performing a post processing, the strength as a nonwoven fabric is weak, therefore, the handleability is poor, and further, there have been problems that fluff is prone to occur, and the like.

Accordingly, for such a nonwoven fabric, in general, a method for solving the problems has been taken by performing a post processing (for example, Japanese Patent Laying-Open No. 2012-41644 (PTD 1)).

However, in the nonwoven fabric that has been subjected to a post processing as described above, at least some parts of the nonwoven fabric have a high density, as a result there may be a case where the performances of the air permeability and the like are affected, therefore, it has been desired to develop a nonwoven fabric that is excellent in the handleability even though there are few high-density parts.

### CITATION LIST

### PATENT DOCUMENT

PTD 1: Japanese Patent Laying-Open No. 2012-41644

### SUMMARY OF INVENTION

### TECHNICAL PROBLEMS

The present invention has been made to solve the above problems, and an object of the present invention is to provide a nonwoven fabric having sufficient strength to be handled alone and including fibers that contain a polymer having a Tg of greater than or equal to 50°C as a main component without performing a post processing such as emboss processing, calender processing, or spunlace processing, and a method for producing the nonwoven fabric.

### SOLUTIONS TO PROBLEMS

The nonwoven fabric of the present invention is a nonwoven fabric according to claim 1, including fibers that contain a polymer having a glass transition temperature of greater than or equal to 50°C as a main component, having a vertical strength of greater than or equal to 1 N/5 cm per 1 g/m², and satisfying the following conditions (1) and (2):
(1) a density is 0.1 to 0.4 g/cm³; and
(2) a proportion of parts with a density exceeding 0.4 g/cm³ is less than or equal to 3% in a cross section in a thickness direction.

It is preferred that the nonwoven fabric of the present invention has a fiber fusion rate of greater than or equal to 15% in a cross section in a thickness direction, and an average area of parts where fibers are fused of less than or equal to 70 µm².

The nonwoven fabric of the present invention preferably has an average fiber diameter of 1 to 10 µm.

The present invention is also to provide a method according to claim 5 for producing the above-described nonwoven fabric of the present invention, in which a melt blown method is performed while maintaining a temperature in at least one of (1) a hemispherical space of 0.5 × collection distance d around a nozzle tip relative to the collection distance d between the tip of a spinning nozzle and a collection surface of spun fibers, and (2) a point of 1 cm from the collection surface on the straight line relative to the collection distance d between the tip of the spinning nozzle and the collection surface of spun fibers at a temperature higher than the glass transition temperature by greater than 15°C to 60°C.

### ADVANTAGEOUS EFFECTS OF INVENTION

According to the present invention, a nonwoven fabric having sufficient strength to be handled alone and including fibers that contain a polymer having a Tg of greater than or equal to 50°C as a main component without performing a post processing such as emboss processing, calender processing, or spunlace processing, and a method for producing the nonwoven fabric can be provided.

### BRIEF DESCRIPTION OF DRAWINGS

Fig. 1 is a scanning electron microscope (SEM) photograph of a cross section in a thickness direction of a nonwoven fabric of the present invention.
Fig. 2 is a schematic diagram for illustrating a principle of a method for producing a nonwoven fabric of the present invention.
Fig. 3 is a schematic diagram for illustrating a principle of the method for producing a nonwoven fabric of the present invention.
Fig. 4 is a diagram schematically showing one preferred example of the method for producing a nonwoven fabric of the present invention.
Fig. 5 is a diagram schematically showing another preferred example of the method for producing a nonwoven fabric of the present invention.
Fig. 6 is a SEM photograph of a cross section in a thickness direction in a case where a nonwoven fabric is formed by a melt blown method using a polymer having a Tg of greater than or equal to 50°C, and then the formed nonwoven fabric is subjected to calender processing as the post processing.
Fig. 7 is a SEM photograph of a cross section in a thickness direction in a case where a nonwoven fabric is formed by a melt blown method using a polymer having a Tg of greater than or equal to 50°C, and then the formed nonwoven fabric is subjected to emboss processing as the post processing.
Fig. 8 is a SEM photograph of a cross section in a thickness direction in a case where a nonwoven fabric is formed by a melt blown method using a polymer having a Tg of greater than or equal to 50°C, and then the formed nonwoven fabric is subjected to spunlace processing as the post processing.

### DESCRIPTION OF EMBODIMENTS

### [1] Nonwoven fabric

The nonwoven fabric of the present invention has a vertical strength (strength in a vertical direction (a direction of flow in producing the nonwoven fabric)) per 1 g/m² of greater than or equal to 1 N/5 cm. According to the present invention, a nonwoven fabric having sufficient strength to be handled alone as a nonwoven fabric can be obtained without performing a post processing such as calender processing, emboss processing, or spunlace processing, which generates a part partially with a high density. The strength of the nonwoven fabric of the present invention is more preferably greater than or equal to 1.2 N/5 cm, and furthermore preferably 1.5 N/5 cm. In a case where a nonwoven fabric is formed by a conventional melt blown method, and the formed nonwoven fabric is not subjected to a post processing such as calender processing, emboss processing, or spunlace processing (Comparative Example 1 described later), the vertical strength per 1 g/m² becomes significantly poor, but even as compared with such a case, the nonwoven fabric of the present invention is a nonwoven fabric significantly excellent in the handleability.

In addition, the nonwoven fabric of the present invention is a nonwoven fabric having a density of 0.1 to 0.4 g/cm³. When the density is greater than or equal to 0.1 g/cm³, preferred form and properties as a nonwoven fabric can be maintained, and when the density is less than or equal to 0.4 g/cm³, desired performance such as high permeability can be easily obtained in the nonwoven fabric. The density of the nonwoven fabric of the present invention is preferably less than or equal to 0.35 g/cm³, and more preferably less than or equal to 0.3 g/cm³, and preferably greater than or equal to 0.1 g/cm³, and more preferably greater than or equal to 0.11 g/cm³.

In addition, in the nonwoven fabric of the present invention, a proportion of parts with a density exceeding 0.4 g/cm³ is less than or equal to 3%. In a case where the proportion of parts with a density exceeding 0.4 g/cm³ exceeds 3%, unevenness is generated on the nonwoven fabric, and as a result, failures that the air permeability is affected, uneven strength is generated, and the like may occur in some cases. The proportion of parts with a density exceeding 0.4 g/cm³ is more preferably less than or equal to 2.5%, and furthermore preferably less than or equal to 2%.

The proportion of parts with a density exceeding 0.4 g/cm³ in the nonwoven fabric described above is determined as follows. Using a SEM, a 100-times magnified photograph of the cross section in the thickness direction of the nonwoven fabric is taken, a straight line of 10 mm of the photograph is observed in the width direction by visual inspection, the length occupied by the parts with a density exceeding 0.4 g/cm³ is measured in this straight line, and the proportion is determined by the following equation: $Proportion \left(%\right) of parts with a density exceeding 0.4 g / {cm}^{3} = length of parts with a density exceeding 0.4 g / {cm}^{3} \left(mm\right) / 10 \left(mm\right) \times 100 .$ Note that with the observation of the photograph, it is determined whether or not the density exceeds 0.4 g/cm³ by using a function of distance measurement between two points attached to the SEM, and by investigating the length occupied by the parts with a density exceeding 0.4 g/cm³.

Herein, Fig. 1 is photographs of a scanning electron microscope (SEM) of a cross section in a thickness direction of the nonwoven fabric of the present invention (Example 1 described later, Fig. 1(a) shows a 100-times magnified photograph, and Fig. 1(b) shows a 1000-times magnified photograph). As shown in Fig. 1, the nonwoven fabric of the present invention has a fusion part 3 in which fibers 2 are partially fused (self-fused) to one another although being a nonwoven fabric 1 including fibers that contain a polymer having a Tg of greater than or equal to 50°C as a main component. Herein, in a cross section in a thickness direction of nonwoven fabric 1 of the present invention, the fiber fusion rate is preferably greater than or equal to 15%, more preferably greater than or equal to 20%, and furthermore preferably greater than or equal to 25%. In a case where the fiber fusion rate is less than 15%, the proportion of the parts where fibers are fused to one another occupied in the nonwoven fabric is extremely low and the strength becomes insufficient, and failures may occur in the handleability, such that the nonwoven fabric cannot be handled alone, in some cases. In addition, if the fiber fusion rate is extremely high, there may be a case where a paper-like seat is formed, the air permeability is affected, or the like, therefore, the fiber fusion rate of a nonwoven fabric is preferably less than or equal to 60%, and more preferably less than or equal to 50%.

The above-described fiber fusion rate of a nonwoven fabric can be calculated, for example, by the following procedures. At first, using a SEM, a 1000-times magnified photograph of the cross section in the thickness direction of the nonwoven fabric is taken, and from the photograph, a proportion of the number of the cut sections where fibers are fused to one another relative to the number of fiber cut sections (fiber cross sections) is determined by visual inspection. The proportion of the number of the cross sections where greater than or equal to two fibers are fused to one another, occupied in the total number of the fiber cross sections that can be found in each region is expressed as a percentage on the basis of the following equation:
Fiber fusion rate (%) = (the number of the cross sections where greater than or equal to two fibers are fused to one another) / (the total number of the fiber cross sections) × 100. Provided that the number of the fibers whose cross sections can be seen is counted in each photograph, and in a case where the number of fiber cross sections are less than or equal to 100, photographs to be observed are added so that the total number of the fiber cross sections exceeds 100. Further, in the parts where fibers are in contact with one another, there are a part where fibers are simply in contact with one another without fusing to one another and a part where fibers are bonded with fusing to one another, and since the nonwoven fabric is cut for the SEM photography, the fibers that are simply in contact with one another are separated due to the stress of each fiber in the cross section. Therefore, in the SEM photograph, it can be determined that fibers, which are in contact with one another, are fused to one another.

Further, in the nonwoven fabric of the present invention, an average area of parts where fibers are fused is preferably less than or equal to 70 µm², and more preferably less than or equal to 50 µm². Herein, as a conventional example, a SEM photograph of a cross section in a thickness direction in a case where a nonwoven fabric formed by a melt blown method has been subjected to a post processing is shown in each of Figs. 6 to 8. Fig. 6 shows SEM photographs in a case where calender processing has been performed as the post processing (Comparative Example 3 described later, Fig. 6(a) shows a 100-times magnified photograph, and Fig. 6(b) shows a 1000-times magnified photograph), Fig. 7 shows SEM photographs in a case where emboss processing has been performed as the post processing (Comparative Example 2 described later, Fig. 7(a) shows a 100-times magnified photograph, and Fig. 7(b) shows a 1000-times magnified photograph), and Fig. 8 shows SEM photographs in a case where spunlace processing has been performed as the post processing (Comparative Example 4 described later, Fig. 8(a) shows a 100-times magnified photograph, and Fig. 8(b) shows a 1000-times magnified photograph). As is prominent in Figs. 6(b) and 7(b), in a nonwoven fabric to which calender processing or emboss processing has been performed as the post processing, a large number of parts where fibers are fused to one another to the extent of the state that discrimination of the fiber diameter becomes difficult are formed, and the average area of parts where fibers are fused exceeds 70 µm². Since the average area of parts where fibers are fused is less than or equal to 70 µm², the nonwoven fabric of the present invention can be distinguished from the nonwoven fabric to which calender processing or emboss processing has been performed as the post processing, as is prominent in Figs. 6(b) and 7(b). On the other hand, as shown in Fig. 8, in the nonwoven fabric to which spunlace processing has been performed, the parts where fibers are fused are extremely few, and the fiber fusion rate becomes less than 15%. As described above, when the fiber fusion rate in a cross section in a thickness direction is greater than or equal to 15%, and an average area of parts where fibers are fused is less than or equal to 70 µm², the nonwoven fabric of the present invention can be clearly distinguished from the nonwoven fabric to which post processing such as calender processing, emboss processing, spunlace processing, or the like has been performed.

It is preferred that the nonwoven fabric of the present invention has an average fiber diameter within the range of 1 to 10 µm. As described above, it is preferred that the nonwoven fabric of the present invention contains a fusion part where fibers are fused to one another, but even in the case, different from the case where calender processing has been performed (see Fig. 6(b)), or the case where emboss processing has been performed (see Fig. 7(b)), the fusion is to the extent that the fiber diameter can be discriminated (Fig. 1(b)), and the average fiber diameter can be calculated. In the nonwoven fabric of the present invention, in a case where the average fiber diameter is less than 1 µm, the discharge amount is required to be decreased, and thus the productivity is lowered, in addition, the discharge pressure becomes unstable, and thread breakage or polymer lumps may be frequently generated and thus the formation of a web may become difficult. Further, in the nonwoven fabric of the present invention, in a case where the average fiber diameter exceeds 10 µm, the denseness may become poor. In particular, for the reason of achieving a balance between the production stability and the denseness, the average fiber diameter of the nonwoven fabric of the present invention is more preferably within the range of 1.2 to 9.5 µm, and particularly preferably within the range of 1.5 to 9.0 µm.

The nonwoven fabric of the present invention includes fibers that contain a polymer having a Tg of greater than or equal to 50°C as a main component.

In the present invention, the expression "fibers that contain a polymer having a Tg of greater than or equal to 50°C as a main component" is referred to as fibers that contain a greater than or equal to 50% by mass of polymer having a Tg of greater than or equal to 50°C, and the content is preferably greater than or equal to 70% by mass, more preferably greater than or equal to 80% by mass, furthermore preferably greater than or equal to 90% by mass, and particularly preferably greater than or equal to 100% by mass.

In addition, when the total of the polymers having a Tg of greater than or equal to 50°C is greater than or equal to 50% by mass, the nonwoven fabric of the present invention may contain greater than or equal to two different polymers having a Tg of greater than or equal to 50°C.

Examples of the polymer used in the present invention and having a Tg of greater than or equal to 50°C include polyamide, polyphenylene sulfide, polyethylene terephthalate, and polycarbonate, and from the viewpoint of combining flame retardancy, heat resistance, and the like, amorphous polyetherimide (PEI) is particularly preferred.

The amorphous PEI used in the present invention is a polymer containing an aliphatic, alicyclic or aromatic ether unit and a cyclic imide as a repeating unit, and is not particularly limited as long as having amorphousness and melt formability. Further, as long as the amorphous PEI is in a range not inhibiting the effect of the present invention, a cyclic imide, and a structural unit other than an ether bond, for example, an aliphatic, alicyclic, or aromatic ester unit, an oxycarbonyl unit, and the like may be contained in the main chain of the amorphous PEI.

As the amorphous PEI used in the present invention, a polymer represented by the following general formula is suitably used. Provided that in the formula, R1 represents a divalent aromatic residue having 6 to 30 carbon atoms, and R2 represents a divalent organic group selected from the group consisting of a divalent aromatic residue having 6 to 30 carbon atoms, an alkylene group having 2 to 20 carbon atoms, a cycloalkylene group having 2 to 20 carbon atoms, and a polydiorganosiloxane group that is chain-stopped by an alkylene group having 2 to 8 carbon atoms.

In addition, in the amorphous PEI used in the present invention, the melt viscosity at 330°C is preferably 100 to 3000 Pa·s. When the melt viscosity of amorphous PEI at 330°C is less than 100 Pa·s, there may be a case where fiber dust, or resin particles called shots that occur due to the failure in formation of fibers are frequently generated during spinning. Further, when the melt viscosity of amorphous PEI at 330°C exceeds 3000 Pa·s, there may be a case where a trouble occurs during polymerization or granulation, for example, ultra-fine fibers are difficult to be formed, and oligomers are generated during polymerization. The melt viscosity at 330°C is preferably 200 to 2700 Pa·s, and more preferably 300 to 2500 Pa·s.

In the amorphous PEI used in the present invention, the glass transition temperature is preferably greater than or equal to 200°C. When the glass transition temperature is less than 200°C, there may be a case where the heat resistance of a nonwoven fabric to be obtained is poor. Further, as the glass transition temperature of amorphous PEI is higher, a nonwoven fabric excellent in the heat resistance can be obtained, therefore, this is preferred, but when the glass transition temperature is extremely high, the fused temperature may also become high, and thus a polymer may be decomposed during fusion. The glass transition temperature of the amorphous PEI is more preferably 200 to 230°C, and furthermore preferably 205 to 220°C.

The molecular weight of the amorphous PEI used in the present invention is not particularly limited, and in consideration of the mechanical properties, the dimensional stability, or the processability of the fibers or nonwoven fabric to be obtained, the weight average molecular weight (Mw) is preferably 1000 to 80000. When amorphous PEI having a high molecular weight is used, the amorphous PEI is excellent in terms of the fiber strength, the heat resistance, and the like, therefore, this is preferred, but from the viewpoint of the cost for producing a resin, the cost for forming into small fibers, and the like, the weight average molecular weight is preferably 2000 to 50000, and more preferably 3000 to 40000.

In the present invention, from the viewpoint of the amorphousness, the melt formability, and the cost, as the amorphous PEI, a condensate of 2,2-bis[4-(2,3-dicarboxyphenoxy)phenyl]propane dianhydride and m-phenylenediamine or p-phenylenediamine, which mainly has a structural unit represented by the following formula, is preferably used. This PEI is commercially available from SABIC Innovative Plastics under the trademark of "ULTEM".

The fibers containing a polymer having a Tg of greater than or equal to 50°C as a main component, which are included in the nonwoven fabric of the present invention, may contain an antioxidant, an antistatic agent, a radical inhibitor, a matting agent, an UV absorber, a flame retardant, an inorganic substance, and the like within the range of not impairing the effects of the present invention. As the specific examples of the inorganic substance, carbon nanotube, fullerene, a silicate such as talc, wollastonite, zeolite, sericite, mica, kaolin, clay, pyrophyllite, silica, bentonite, and alumina silicate, a metal oxide such as silicon oxide, magnesium oxide, alumina, zirconium oxide, titanium oxide, and iron oxide, a carbonate such as calcium carbonate, magnesium carbonate, and dolomite, a sulfate such as calcium sulfate, and barium sulfate, a hydroxide such as calcium hydroxide, magnesium hydroxide, and aluminum hydroxide, glass beads, glass flakes, glass powder, ceramic beads, boron nitride, silicon carbide, carbon black, graphite, and the like are used. Further, for the purpose of improving the hydrolysis resistance of fibers, a terminal sequestering agent such as a mono- or di-epoxy compound, a mono- or poly-carbodiimide compound, a mono- or di-oxazoline compound, and a mono- or di-azirine compound may be contained.

Furthermore, the nonwoven fabric of the present invention may include fibers other than the fibers that contain a polymer having a Tg of greater than or equal to 50°C as a main component, for example, fibers made of polyethylene, polypropylene, ethylene vinyl acetate, or the like within the range of not impairing the effects of the present invention. The content of the fibers that contain a polymer having a Tg of greater than or equal to 50°C as a main component is not particularly limited, and is preferably greater than or equal to 50% by mass, more preferably greater than or equal to 70% by mass, furthermore preferably greater than or equal to 90% by mass, and particularly preferably 100% by mass.

The thickness of the nonwoven fabric of the present invention is not particularly limited, and is preferably within the range of 10 to 1000 µm, more preferably within the range of 15 to 500 µm, and particularly preferably within the range of 20 to 200 µm. In a case where the thickness of the nonwoven fabric is less than 10 µm, the strength may be lowered, and breakage may occur during processing, and further, in a case where the thickness of the nonwoven fabric of the present invention exceeds 1000 µm, the formation of a web may become difficult.

In addition, in the nonwoven fabric of the present invention, the air permeability is preferably greater than or equal to 10 cc/cm²/sec, and more preferably greater than or equal to 20 cc/cm²/sec, and further preferably less than or equal to 130 cc/cm²/sec, and more preferably less than or equal to 120 cc/cm²/sec. By setting the air permeability within the range described above, the nonwoven fabric of the present invention can be suitably used for the application of a filter or the like.

In addition, the basis weight of the nonwoven fabric of the present invention is not particularly limited, and is preferably within the range of 10 to 1000 g/m², and more preferably within the range of 15 to 500 g/m². In a case where the basis weight of the nonwoven fabric is less than 10 g/m², the strength may be lowered, and breakage may occur during processing, and further, in a case where the basis weight of the nonwoven fabric exceeds 1000 g/m², the case is not preferred from the viewpoint of the productivity.

### [2] Method for producing nonwoven fabric

The present invention is also to provide a method for producing the above-described nonwoven fabric of the present invention. Note that the above-described nonwoven fabric of the present invention is a nonwoven fabric including fibers that contain a polymer having a Tg of greater than or equal to 50°C as a main component, and having a vertical strength of greater than or equal to 1 N/5 cm per 1 g/m². As long as the density is 0.1 to 0.4 g/cm³, and the proportion of parts with a density exceeding 0.4 g/cm³ is less than or equal to 3% in a cross section in a thickness direction, the nonwoven fabric of the present invention may be a nonwoven fabric produced by the method for producing a nonwoven fabric of the present invention, or may be a nonwoven fabric not produced by the method for producing a nonwoven fabric of the present invention, but a nonwoven fabric produced by the method for producing a nonwoven fabric of the present invention is preferred.

The method for producing a nonwoven fabric of the present invention is characterized in that a melt blown method is performed while maintaining a temperature in at least one of the following (1) and (2) at a temperature higher than the Tg of the polymer to be a main component by greater than or equal to 10°C.
(1) A hemispherical space of 0.5 × collection distance d around a nozzle tip relative to the collection distance d between the tip of a spinning nozzle and a collection surface of spun fibers.
(2) A point of 1 cm from the collection surface on the straight line relative to the collection distance d between the tip of the spinning nozzle and the collection surface of spun fibers.

Note that in a case where greater than or equal to two different kinds of polymers having a Tg of greater than or equal to 50°C are used, the temperature is maintained at a temperature higher than the Tg of the polymer having the highest Tg by greater than or equal to 10°C.

Herein, Figs. 2 and 3 are schematic diagrams for illustrating a principle of the method for producing a nonwoven fabric of the present invention. Fig. 2 shows a state that a melt blown method is performed by using a melt blown device 11, and after polymer fibers 13 are discharged (spun) from a spinning nozzle 12 of melt blown device 11, discharged (spun) polymer fibers 13 are collected by a rotating roll 14, and a web (that is in a sheet shape obtained by piling up fibers) 15 is formed. Hot air (primary air) 16 for spinning is discharged together with polymer fibers 13 from spinning nozzle 12 of melt blown device 11, and flows along the curved surface of roll 14. At that time, the present inventors found that as cold air flows as accompanying flow 17 toward spinning nozzle 12, polymer fibers 13 discharged from a tip 12a of spinning nozzle 12 are rapidly cooled before reaching a surface (collection surface of spun fibers) 14a of roll 14, and thus web 15 having low strength and poor handleability is formed. For this reason, conventionally, it has been required to perform a post processing such as calender processing, emboss processing, or spunlace (hydroentangle) processing to impart strength to a web and to form a nonwoven fabric. The temperature of the primary air (measured using a contact-type temperature sensor) discharged from a tip of a spinning nozzle, which was actually measured by the present inventors, was 420°C, but the temperature of the primary air (measured using a contact-type temperature sensor) reached a collection surface of spun fibers was 145°C.

In the method for producing a nonwoven fabric of the present invention, as shown in Fig. 3, a temperature in a hemispherical space A of 0.5 × collection distance d around a nozzle tip relative to the collection distance d between tip 12a of spinning nozzle 12 and collection surface 14a of spun fibers 13, a radius x around tip 12a of spinning nozzle 12 being 0.5 × collection distance d, and/or a temperature in a point B (not shown) of 1 cm from the collection surface on the straight line relative to the direct distance d between tip 12a of spinning nozzle 12 and collection surface 14a of spun fibers 13 maintains at a temperature higher than the Tg of the polymer by greater than or equal to 10°C. Herein, in the method for producing a nonwoven fabric of the present invention, the temperature in either space A or point B is only required to be maintained at a temperature higher than the Tg of the polymer by greater than or equal to 10°C, but the temperatures in both of space A and point B may be maintained at a temperature higher than the Tg of the polymer by greater than or equal to 15°C. Further, as in the example shown in Fig. 3, a part of space A and a part of point B may be overlapped.

By maintaining the temperature in at least one of the above-described space A and point B at a temperature higher than the Tg by greater than or equal to 10°C, the cooling of primary air by the accompanying flow as described above is prevented, and the nonwoven fabric of the present invention that contains a polymer having a Tg of greater than or equal to 50°C as a main component and has sufficient strength obtained by fusing fibers to one another can be produced without performing a post processing such as calender processing, emboss processing, or spunlace processing (that is, web 15 collected by roll 14 can be used as it is as the nonwoven fabric).

Herein, in a case where a temperature in hemispherical space A of radius x that is 0.5 × collection distance d around a nozzle tip relative to the collection distance d between tip 12a of spinning nozzle 12 and collection surface 14a of spun fibers 13 is higher than the Tg by greater than or equal to 10°C, the temperature in a space around hemispherical space A is not particularly limited. Radius x in hemispherical space A around tip 12a of spinning nozzle 12 is preferably 3 to 12 cm, and particularly preferably 5 cm. For example, a temperature in space A can be measured by arranging, for example, a thermocouple-type thermometer as a thermometer at any position on a curved surface constituting a hemisphere assumed as a boundary of space A.

Further, even in a case where a temperature in point B of 1 cm from the collection surface on the straight line relative to the direct distance d between tip 12a of spinning nozzle 12 and collection surface 14a of spun fibers 13 is higher by greater than or equal to 10°C, the temperature in a space around point B is not particularly limited.

In the method for producing a nonwoven fabric of the present invention, the temperature in at least one of space A and point B is maintained so as to be at a temperature higher than the Tg of a polymer by greater than 15 to 60°C). In a case where a temperature in at least one of space A and point B is at a temperature less than or equal to the Tg of a polymer, or is less than 10°C even if being higher than the Tg, the effect of preventing the cooling of the spun fibers by the accompanying flow is insufficient, and thus a nonwoven fabric having low strength and poor handleability may be produced.

Fig. 4 is a diagram schematically showing one preferred example of the method for producing a nonwoven fabric of the present invention. In the example shown in Fig. 4, a hot air injection device 21 is arranged in the vicinity of tip 12a of spinning nozzle 12 so as to blow hot air (for the primary air described above, this hot air is referred to as "secondary air") 22 toward tip 12a of spinning nozzle 12. The arrangement of hot air injection device 21 is not particularly limited, and hot air injection device 21 in a shape of continuously forming a circumference surrounding tip 12a of spinning nozzle 12 may be arranged so that a blowing tip is directed toward tip 12a of spinning nozzle 12, or multiple hot air injection devices 21 may be arranged around tip 12a so that a blowing tip is directed toward tip 12a of spinning nozzle 12. For example, in this way, as described above, by maintaining the temperature in at least one of the above (1) and (2) at a temperature higher than the Tg of a polymer by greater than or equal to 10°C, a melt blown method can be performed. Note that as hot air injection device 21, a conventionally known appropriate hot air injection device can be used without any particular limitation.

The temperature of secondary air 22 injected so as to be blown into tip 12a of spinning nozzle 12 by hot air injection device 21 is not particularly limited as long as the temperature in at least one of the above (1) and (2) (in particular, a space of the above-described (1)) can be maintained at a temperature higher than the Tg of a polymer by greater than or equal to 30°C, and is preferably at a temperature higher than the Tg of a polymer by 35 to 70°C and more preferably at a temperature higher than the Tg of a polymer by 35 to 60°C. In a case where the temperature of secondary air 22 is at a temperature higher than the Tg of a polymer by less than 30°C, it becomes difficult to maintain the temperature in at least one of the above-described (1) and (2) (in particular, a space of the above-described (1)), and further, there is a tendency that the fiber fusion is small and the nonwoven fabric strength is weak. Furthermore, in a case where the temperature of secondary air 22 is higher than the Tg of a polymer by exceeding 70°C, there is a tendency that the fiber fusion is increased and a paper-like nonwoven fabric is obtained. Moreover, the flow rate of secondary air 22 is also not particularly limited as long as the temperature in at least one of the above (1) and (2) (in particular, a space of the above-described (1)) can be maintained at a temperature higher than the Tg of a polymer by greater than or equal to 10°C, and is in order not to disturb the flow of the primary air, preferably within the range of 3 to 12 Nm³/m, and more preferably within the range of 4 to 10 Nm³/m.

Fig. 5 is a diagram schematically showing another preferred example of the method for producing a nonwoven fabric of the present invention. In the example shown in Fig. 5, at least a part of a space between tip 12a of spinning nozzle 12 and collection surface 14a of spun fibers is covered with a cover 31. As a result, the primary air discharged from tip 12a of the spinning nozzle 12 stays in the space covered with cover 31 as circulation air 32, and thus the primary air discharged from tip 12a of spinning nozzle 12 is not rapidly cooled by the accompanying flow as in a case of not being covered with cover 31. As described above, also in this way, by maintaining the temperature in at least one of the above (1) and (2) at a temperature higher than the Tg of a polymer by greater than or equal to 10°C, a melt blown method can be performed. Note that as long as the temperature in at least one of the above (1) and (2) is maintained at a temperature higher than the Tg of a polymer by greater than or equal to 10°C, cover 31 does not need to cover throughout between tip 12a of spinning nozzle 12 and collection surface 14a of spun fibers. As in the example shown in Fig. 5, it is preferred that cover 31 is arranged so as to cover throughout between tip 12a of spinning nozzle 12 and collection surface 14a of spun fibers. A material for forming such cover 31 is not particularly limited as long as having heat resistance to the extent that the cover is not deteriorated due to the temperature of primary air, for example, a metal such as steel use stainless (SUS), aluminum, and copper can be mentioned, and SUS is preferred from the viewpoint of the durability, the processability, and the heat resistance.

In the method for producing a nonwoven fabric of the present invention, by maintaining the temperature in at least one of the above (1) and (2) at a temperature higher than the Tg of a polymer by greater than or equal to 10°C, a melt blown method is performed, and processes, conditions, and the like that are similar to those in a conventional melt blown method can be suitably adopted except that a post processing such as calender processing, emboss processing, or spunlace processing is not performed. As the spinning conditions, for example, a spinning temperature of 300 to 500°C, a hot air temperature (primary air temperature) of 300 to 500°C, and an amount of air of 5 to 25 Nm³ per 1 m of nozzle length can be mentioned as suitable examples, but of course, the spinning conditions are not limited to these examples.

### EXAMPLES

Hereinafter, the present invention will be specifically described with reference to examples, however, the present invention is not limited to the following examples at all.

### [Density of nonwoven fabric (g/cm³)]

The volume of a nonwoven fabric was measured using [basis weight of the nonwoven fabric] and [thickness of the nonwoven fabric], and from these results, the density of the nonwoven fabric was calculated.

### [Proportion (%) of parts with a density exceeding 0.4 g/cm³]

Using a scanning electron microscope, a 100-times magnified photograph of a cross section in a thickness direction of a nonwoven fabric was taken, a straight line of 10 mm of the photograph was observed in a width direction by visual inspection, the length occupied by parts with a density exceeding 0.4 g/cm³ was measured in this straight line, and a proportion was determined by the following equation: $Proportion \left(%\right) of parts with a density exceeding 0.4 g / {cm}^{3} = length of parts with a density exceeding 0.4 g / {cm}^{3} \left(mm\right) / 10 \left(mm\right) \times 100 .$ Note that with the observation of the photograph, it was determined whether or not the density exceeds 0.4 g/cm³ by using a function of distance measurement between two points attached to the SEM, and by investigating the length of the parts with a density exceeding 0.4 g/cm³.

### [Vertical strength (strength in vertical direction (direction of flow), N/5 cm)]

The nonwoven fabric was cut into a piece with a width of 5 cm, and the piece was extended at a tensile rate of 10 cm/min by using an autograph manufactured by Shimadzu Corporation in accordance with JIS L 1906, and the load value at the time of breaking was defined as the vertical strength.

### [Melt viscosity]

The melt viscosity was measured under conditions of a temperature of 330°C and a shear rate r = 1200 sec⁻¹, by using Capilograph 1B of Toyo Seiki Seisaku-Sho, Ltd.

### [Glass transition temperature (°C)]

By using a solid dynamic viscoelasticity measuring device, "Rheospectra DVE-V4" manufactured by Rheology Co. Ltd., the temperature dependency of loss tangent (tan δ) was measured at a frequency of 10 Hz and at a temperature rise rate of 10°C/min, and the glass transition temperature was determined from the peak temperature. Herein, the peak temperature of tan δ means a temperature at which the first derivative value of the amount of change to the temperature of the value of tan δ becomes zero.

### [Fiber fusion rate (%)]

Using a scanning electron microscope, a 1000-times magnified photograph of a cross section in a thickness direction of a nonwoven fabric was taken, and from the photograph, a proportion of the number of cut sections where fibers are fused to one another relative to the number of fiber cut sections (fiber cross sections) was determined by visual inspection. A proportion of the number of the cross sections where greater than or equal to two fibers are fused to one another, occupied in the total number of the fiber cross sections that can be found in each region was expressed as a percentage on the basis of the following equation: $Fiber fusion rate \left(%\right) = \left(the number of the cross sections where greater than or equal to two fibers are fused\right) / \left(the total number of the fiber cross sections\right) \times 100 .$ Provided that the number of the fibers whose cross sections can be seen is counted in each photograph, and in a case where the number of fiber cross sections are less than or equal to 100, photographs to be observed were added so that the total number of the fiber cross sections exceeds 100.

### [Average area of parts where fibers are fused]

Using a scanning electron microscope, a 1000-times magnified photograph of the cross section in the thickness direction of the nonwoven fabric was taken, from this photograph, the area of the parts where fibers are fused was calculated, and the total was divided by the number of the parts where fibers are fused to obtain the average value.

### [Average fiber diameter (µm)]

The nonwoven fabric was photographed with magnification by a scanning electron microscope, the diameters of arbitrary 100 fibers were measured, the average value was calculated, and defined as the average fiber diameter.

### [Basis weight of nonwoven fabric (g/m²)]

In accordance with JIS L 1913, a sample piece of length 20 cm × width 20 cm was taken, the mass was measured with an electronic balance, the measured mass was divided by the test piece area 400 cm², and the mass per unit area was defined as the basis weight.

### [Thickness of nonwoven fabric (µm)]

In accordance with JIS L 1913, by using the same sample pieces as those in the measurement of basis weight, the thickness was measured at five positions in each sample piece with a digital thickness measuring device having a diameter of 16 mm and a load of 20 gf/cm² (B1 type, manufactured by Toyo Seiki Seisaku-Sho, Ltd.), and the average value of the thicknesses at 15 positions was defined as the thickness of the sheet.

### [Air permeability of nonwoven fabric (cc/cm²/sec)]

The air permeability was measured in accordance with a fragile form method of JIS L 1913 "Test methods for nonwovens".

### <Example 1>

Amorphous polyetherimide having a melt viscosity at 330°C of 500 Pa·s was used, and extruded with an extruder to be supplied to a melt blown device having a nozzle with a nozzle hole diameter D (diameter) of 0.3 mm, L (nozzle length) / D = 10, and a nozzle hole pitch of 0.75 mm. By blowing hot air to the amorphous polyetherimide at a single hole discharge rate of 0.09 g/min, a spinning temperature of 390°C, a hot air (primary air) temperature of 420°C, and 10 Nm³/min per 1 m of nozzle width, a nonwoven fabric having a basis weight of 25 g/m² was produced. At this time, a hot air injection device as in the example shown in Fig. 4 was arranged so that hot air (secondary air) blows into a tip of the spinning nozzle of the melt blown device, and hot air (secondary air) at a temperature of 260°C was blown at a flow rate of 2 Nm³ toward the tip of the spinning nozzle. The direct distance d between the tip of the spinning nozzle and a receiving surface of a roller receiving the spun fibers was 10 cm, and the temperature measured by a thermometer (AD-5601A (manufactured by A&D Company, Limited)) arranged so as to be positioned on a hemispherical outer periphery of a radius x = 5 cm around the tip of the spinning nozzle was 235°C (that is, space A was maintained at a temperature higher than 215°C that is a glass transition temperature of the amorphous PEI by 20°C). Further, the temperature measured by a thermometer (AD-5601A (manufactured by A&D Company, Limited)) arranged so as to be positioned 1 cm from a collection surface on the straight line relative to the direct distance d between the tip of the spinning nozzle and the collection surface of the spun fibers was 242°C (that is, point B was maintained at a temperature higher than 215°C that is a glass transition temperature of the amorphous PEI by 27°C). In this way, a nonwoven fabric was obtained without performing a post processing. As a SEM photograph of a cross section in a thickness direction of the obtained nonwoven fabric, a 100-times magnified photograph is shown in Fig. 1(a), and a 1000-times magnified photograph is shown in Fig. 1(b).

### <Example 2>

A nonwoven fabric was obtained by using amorphous polyetherimide having a melt viscosity at 330°C of 900 Pa·s in the similar manner as in Example 1 except that the spinning temperature was 420°C, the average fiber diameter was 3.7 µm, and the temperature measured by a thermometer positioned on a hemispherical outer periphery of a radius x = 5 cm around the tip of the spinning nozzle was 253°C (that is, space A was maintained at a temperature higher than 215°C that is a glass transition temperature of the amorphous PEI by 38°C), and the temperature measured by a thermometer arranged so as to be positioned 1 cm from the collection surface on the straight line relative to the direct distance d between the tip of the spinning nozzle and the collection surface of the spun fibers was 261°C (that is, point B was maintained at a temperature higher than 215°C that is a glass transition temperature of the amorphous PEI by 46°C).

### <Example 3>

A nonwoven fabric was obtained in the similar manner as in Example 2 except that the basis weight was changed to 10 g/m².

### <Example 4>

Amorphous polycarbonate having a melt viscosity at 300°C of 100 Pa·s was used, and extruded with an extruder to be supplied to a melt blown device having a nozzle with a nozzle hole diameter D (diameter) of 0.3 mm, L (nozzle length) / D = 10, and a nozzle hole pitch of 0.75 mm. By blowing hot air to the amorphous polycarbonate at a single hole discharge rate of 0.09 g/min, a spinning temperature of 340°C, a hot air (primary air) temperature of 370°C, and 10 Nm³/min per 1 m of nozzle width, a nonwoven fabric having a basis weight of 25 g/m² was produced. At this time, a hot air injection device as in the example shown in Fig. 4 was arranged so that hot air (secondary air) blows into a tip of the spinning nozzle of the melt blown device, and hot air (secondary air) at a temperature of 210°C was blown at a flow rate of 2 Nm³ toward the tip of the spinning nozzle. The direct distance d between the tip of the spinning nozzle and a receiving surface of a roller receiving the spun fibers was 10 cm, and the temperature measured by a thermometer (AD-5601A (manufactured by A&D Company, Limited)) arranged so as to be positioned on a hemispherical outer periphery of a radius x = 5 cm around the tip of the spinning nozzle was 185°C (that is, space A was maintained at a temperature higher than 135°C that is a glass transition temperature of the amorphous polycarbonate by 50°C). Further, the temperature measured by a thermometer (AD-5601A (manufactured by A&D Company, Limited)) arranged so as to be positioned 1 cm from the collection surface on the straight line relative to the direct distance d between the tip of the spinning nozzle and a collection surface of the spun fibers was 192°C (that is, point B was maintained at a temperature higher than 135°C that is a glass transition temperature of the amorphous polycarbonate by 57°C).

### <Comparative Example 1>

A nonwoven fabric was obtained in the similar manner as in Example 2 except that the hot air injection device was not arranged (the temperature measured by a thermometer positioned on a hemispherical outer periphery of a radius x = 5 cm around the tip of the spinning nozzle was 41°C, and the temperature measured by a thermometer arranged so as to be positioned 1 cm from the collection surface on the straight line relative to the direct distance d between the tip of the spinning nozzle and the collection surface of the spun fibers was 110°C).

### <Comparative Example 2>

By using an embossing device, the nonwoven fabric obtained in Comparative Example 1 was subjected to emboss processing as the post processing with an embossing roll having a lattice pattern under the conditions of a roll temperature of 180°C, a linear pressure of 50 kg/cm, and a speed of 1 m/min. As a SEM photograph of a cross section in a thickness direction of the obtained nonwoven fabric, a 100-times magnified photograph is shown in Fig. 7(a), and a 1000-times magnified photograph is shown in Fig. 7(b).

### <Comparative Example 3>

By using a calender processing device (iron roll), the nonwoven fabric obtained in Comparative Example 1 was subjected to calender processing as the post processing under the conditions of a roll temperature of 180°C, a linear pressure of 216 kg/cm, and a speed of 3.2 m/min. As a SEM photograph of a cross section in a thickness direction of the obtained nonwoven fabric, a 100-times magnified photograph is shown in Fig. 6(a), and a 1000-times magnified photograph is shown in Fig. 6(b).

### <Comparative Example 4>

By using a hydroentangling device, the nonwoven fabric obtained in Comparative Example 1 was subjected to hydroentangling as the post processing at a speed of 5.0 m/min using a nozzle having a hole diameter of 0.1 mmφ with hydroentangling treatment at three stages of 0.5 MPa, 2.0 MPa, and 2.5 MPa. As a SEM photograph of a cross section in a thickness direction of the obtained nonwoven fabric, a 100-times magnified photograph is shown in Fig. 8(a), and a 1000-times magnified photograph is shown in Fig. 8(b).

### <Comparative Example 5>

A nonwoven fabric was obtained under the similar conditions as in Example 2 except that the temperature of the hot air (secondary air) was changed to 240°C. The temperature measured by a thermometer positioned on a hemispherical outer periphery of a radius x = 5 cm around the tip of the spinning nozzle was 220°C, and the temperature measured by a thermometer arranged so as to be positioned 1 cm from the collection surface on the straight line relative to the direct distance d between the tip of the spinning nozzle and the collection surface of the spun fibers was 217°C.

The results are shown in Tables 1 and 2.

**[Table 1]**

| | Example 1 | Example 2 | Example 3 | Example 4 |
|---|---|---|---|---|
| (Raw material forming nonwoven fabric and production conditions) | | | | |
| Polymer composition of fibers | PEI | PEI | PEI | PC |
| Melt viscosity (Pa•s): 330°C (300°C in Example 4) | 500 | 900 | 900 | 100 |
| Glass transition temperature (°C) | 215 | 215 | 215 | 135 |
| Spinning temperature (°C) | 390 | 420 | 420 | 340 |
| Hot air injection device | Yes | Yes | Yes | Yes |
| Hot air (secondary air) temperature (°C) | 260 | 260 | 260 | 210 |
| Collection distance (cm) | 10 | 10 | 10 | 10 |
| Temperature in space A (°C) | 235 | 253 | 253 | 185 |
| Temperature in point B (°C) | 242 | 261 | 261 | 192 |
| Post processing | No | No | No | No |

| (Performance of nonwoven fabric) | | | | |
|---|---|---|---|---|
| Density (g/cm³) | 0.147 | 0.132 | 0.103 | 0.295 |
| Proportion of parts with a density exceeding 0.4 g/cm³ (%) | 0 | 0 | 0 | 1.4 |
| Vertical strength per 1 g/m² (N/5cm) | 1.6 | 1.7 | 1.6 | 1.9 |
| Fiber fusion rate (%) | 36 | 28 | 28 | 48 |
| Average area of parts where fibers are fused (µm²) | 24 | 33 | 33 | 52 |
| Average fiber diameter (µm) | 2.5 | 3.7 | 3.7 | 2.8 |
| Basis weight (g/m²) | 25 | 25 | 10 | 25 |
| Thickness (µm) | 170 | 189 | 107 | 85 |
| Air permeability (cc/cm²/see) | 54 | 75 | 110 | 32 |

**[Table 2]**

| | Comparative Example 1 | Comparative Example 2 | Comparative Example 3 | Comparative Example 4 | Comparative Example 5 |
|---|---|---|---|---|---|
| (Raw material forming nonwoven fabric and production conditions) | | | | | |
| Polymer composition of fibers | PEI | PEI | PEI | PEI | PEI |
| Melt viscosity (Pa•s): 330°C | 900 | 900 | 900 | 900 | 900 |
| Glass transition temperature (°C) | 215 | 215 | 215 | 215 | 215 |
| Spinning temperature (°C) | 420 | 420 | 420 | 420 | 420 |
| Hot air injection device | No | No | No | No | Yes |
| Hot air (secondary air) temperature (°C) | - | - | - | - | 240 |
| Collection distance (cm) | 10 | 10 | 10 | 10 | 10 |
| Temperature in space A (°C) | 41 | 41 | 41 | 41 | 220 |
| Temperature in point B (°C) | 110 | 110 | 110 | 110 | 217 |
| Post processing | No | Emboss | Calender | Spunlace | No |

| (Performance of nonwoven fabric) | | | | | |
|---|---|---|---|---|---|
| Density (g/cm³) | 0.059 | 0.139 | 0.735 | 0.106 | 0.080 |
| Proportion of parts with a density exceeding 0.4 g/cm³ (%) | 0 | 23 | 100 | 0 | 0 |
| Vertical strength per 1 g/m² (N/5cm) | 0.1 | 0.6 | 0.9 | 0.9 | 0.2 |
| Fiber fusion rate (%) | 0 | 6 | 70 | 0 | 12 |
| Average area of parts where fibers are fused (µm²) | No fiber fusion | 85 | 130 | No fiber fusion | No fiber fusion |
| Average fiber diameter (µm) | 3.7 | 3.7 | 3.7 | 3.7 | 4.0 |
| Basis weight (g/m²) | 25 | 25 | 25 | 25 | 25 |
| Thickness (µm) | 423 | 180 | 34 | 236 | 311 |
| Air permeability (cc/cm²/sec) | 221 | 25 | 4 | 76 | 156 |

### INDUSTRIAL APPLICABILITY

The nonwoven fabric of the present invention is excellent in the handleability in spite of having a low density, therefore, not only can be used in combination with various substrates and other nonwoven fabrics, but also can be used for filters and the like that are required to have permeability.

### REFERENCE SIGNS LIST

1: Nonwoven fabric, 2: fibers, 3: fusion part, 11: melt blown device, 12: spinning nozzle, 12a: tip of spinning nozzle 12, 13: spun amorphous polymer-based fibers, 14: roll, 14a: roll receiving surface, 15: nonwoven fabric, 16: primary air, 17: accompanying flow, 21: hot air injection device, 22: secondary air, 31: cover, 32: circulation air.

## Claims

1. A nonwoven fabric, comprising fibers containing a polymer having a glass transition temperature of greater than or equal to 50°C as a main component, having a vertical strength of greater than or equal to 1 N/5 cm per 1 g/m², and satisfying the following conditions (1) and (2): (1) a density of 0.1 to 0.4 g/cm³; and (2) a proportion of parts with a density exceeding 0.4 g/cm³ of less than or equal to 3% in a cross section in a thickness direction,
wherein the vertical strength is measured as follows: the nonwoven fabric is cut into a piece with a width of 5 cm, and the piece is extended at a tensile rate of 10 cm/min by using an autograph manufactured by Shimadzu Corporation in accordance with JIS L 1906, and a load value at a time of breaking is defined as the vertical strength, and
wherein the proportion of parts with a density exceeding 0.4 g/cm³ is measured as follows: using a scanning electron microscope, a 100-times magnified photograph of a cross section in a thickness direction of the nonwoven fabric is taken, a straight line of 10 mm of the photograph is observed in a width direction by visual inspection, a length occupied by parts with a density exceeding 0.4 g/cm³ is measured in this straight line, and the proportion is determined by the following equation: $proportion \left(%\right) of parts with a density exceeding 0.4 g / {cm}^{3} = length of parts with a density exceeding 0.4 g / {cm}^{3} \left(mm\right) / 10 \left(mm\right) ∗ 100 ,$ with the observation of the photograph, it is determined whether or not the density exceeds 0.4 g/cm³ by using a function of distance measurement between two points attached to the SEM, and by investigating the length of the parts with a density exceeding 0.4 g/cm³.

2. The nonwoven fabric according to claim 1, wherein a fiber fusion rate in a cross section in a thickness direction is greater than or equal to 15%, and an average area of parts where fibers are fused is less than or equal to 70 µm²,
wherein the fiber fusion rate is measured as follows: using a scanning electron microscope, a 1000-times magnified photograph of a cross section in a thickness direction of the nonwoven fabric is taken, and from the photograph, a proportion of a number of the cross sections where greater than or equal to two fibers are fused to one another relative to a total number of the fiber cross sections found in each region is determined by visual inspection and expressed as a percentage on the basis of the following equation: $fiber fusion rate % = \left(the number of the cross sections where greater than or equal to two fibers are fused\right) / \left(the total number of the fiber cross sections\right) \times 100 ,$
provided that the number of the fibers whose cross sections are seen is counted in each photograph, and in a case where the number of fiber cross sections are less than or equal to 100, photographs to be observed are added so that the total number of the fiber cross sections exceeds 100, and
wherein the average area of parts where fibers are fused is measured as follows: using a scanning electron microscope, a 1000-times magnified photograph of a cross section in a thickness direction of the nonwoven fabric is taken, from this photograph, an area of the parts where fibers are fused is calculated, and is divided by a number of the parts where fibers are fused to obtain the average value.

3. The nonwoven fabric according to claim 1, wherein an average fiber diameter is 1 to 10 µm.

4. The nonwoven fabric according to claim 1, wherein amorphous polyetherimide-based fibers are contained.

5. A method for producing the nonwoven fabric according to any one of claims 1 to 4 comprising performing a melt blown method while maintaining a temperature in at least one of (1) a hemispherical space of 0.5 × collection distance d around a nozzle tip relative to the collection distance d between the tip of a spinning nozzle and a collection surface of spun fibers, and (2) a point of 1 cm from the collection surface on a straight line relative to the collection distance d between the tip of the spinning nozzle and the collection surface of spun fibers at a temperature higher than the glass transition temperature by greater than 15°C to 60°C.

## Patentansprüche

1. Vliesstoff, der Fasern aufweist, die ein Polymer mit einer Glasübergangstemperatur von mindestens 50 °C als Hauptkomponente enthalten, der eine senkrechte Festigkeit von mindestens 1 N/5 cm pro 1 g/m² aufweist und die folgenden Bedingungen (1) und (2) erfüllt: (1) eine Dichte von 0,1 bis 0,4 g/cm³ und (2) einen Anteil von Teilen mit einer Dichte von über 0,4 g/cm³ von höchstens 3 % in einem Querschnitt in einer Dickenrichtung, wobei die senkrechte Festigkeit wie folgt gemessen wird: der Vliesstoff wird in ein Stück mit einer Breite von 5 cm geschnitten und das Stück wird mit einer Zugrate von 10 cm/min nach JIS L 1906 mit einem Autograph-Prüfgerät gedehnt, das von der Shimadzu Corporation hergestellt wurde, wobei ein Lastwert zu einer Bruchzeit als senkrechte Festigkeit definiert wird, und
wobei der Anteil von Teilen mit einer Dichte von über 0,4 g/cm³ wie folgt gemessen wird: mit einem Rasterelektronenmikroskop wird ein 100-fach vergrößertes Foto eines Querschnitts des Vliesstoffs in einer Dickenrichtung aufgenommen, eine Gerade von 10 mm aus dem Foto durch Sichtprüfung in einer Breitenrichtung betrachtet, eine von Teilen mit einer Dichte von über 0,4 g/cm³ belegte Länge auf dieser Geraden gemessen und der Anteil durch die folgende Gleichung bestimmt: $Anteil \left(%\right) von Teilen mit einer Dichte über 0,4 g / {cm}^{3} = Länge von Teilen mit einer Dichte über 0,4 g / {cm}^{3} \left(mm\right) / 10 \left(mm\right) \times 100 ,$ wobei bei Betrachtung des Fotos mit einer am REM vorgesehenen Funktion zur Entfernungsmessung zwischen zwei Punkten bestimmt wird, ob die Dichte über 0,4 g/cm³ beträgt, und die Länge der Teile mit einer Dichte über 0,4 g/cm³ ermittelt wird.

2. Vliesstoff nach Anspruch 1, wobei eine Faserfusionsrate in einem Querschnitt in einer Dickenrichtung mindestens 15 % und eine durchschnittliche Fläche von Teilen, in denen Fasern verschmolzen sind, höchstens 70 µm² beträgt,
wobei die Faserfusionsrate wie folgt gemessen wird: mit einem Rasterelektronenmikroskop wird ein 1000-fach vergrößertes Foto eines Querschnitts des Vliesstoffs in einer Dickenrichtung aufgenommen, aus dem durch Sichtprüfung ein Anteil einer Anzahl der Querschnitte, in denen zwei oder mehr Fasern miteinander verschmolzen sind, zu einer Gesamtzahl der in den einzelnen Regionen festgestellten Faserquerschnitte bestimmt und als Prozentwert auf Basis der folgenden Gleichung ausgedrückt wird: $Faserfusionsrate ⁢ % = \left(Anzahl der Querschnitte, in denen zwei oder mehr Fasern verschmolzen sind\right) / \left(Gesamtzahl der Faserquerschnitte\right) \times 100 ,$ und zwar unter der Voraussetzung, dass die Anzahl der Fasern, deren Querschnitte gesehen werden, in den einzelnen Fotos gezählt wird und bei einer Anzahl von Faserquerschnitten von höchstens 100 weitere zu betrachtende Fotos hinzugefügt werden, so dass die Gesamtzahl der Faserquerschnitte über 100 liegt, und
wobei die durchschnittliche Fläche von Teilen, in denen Fasern verschmolzen sind, wie folgt gemessen wird: mit einem Rasterelektronenmikroskop wird ein 1000-fach vergrößertes Foto eines Querschnitts des Vliesstoffs in einer Dickenrichtung aufgenommen und aus diesem Foto eine Fläche der Teile, in denen Fasern verschmolzen sind, berechnet und durch eine Anzahl von Teilen, in denen Fasern verschmolzen sind, geteilt, um den Durchschnittswert zu erhalten.

3. Vliesstoff nach Anspruch 1, wobei ein durchschnittlicher Faserdurchmesser zwischen 1 und 10 µm beträgt.

4. Vliesstoff nach Anspruch 1, wobei amorphe Fasern auf Polyetherimidbasis enthalten sind.

5. Verfahren zum Herstellen des Vliesstoffs nach einem der Ansprüche 1 bis 4, das das Ausführen eines Melt-Blown-Verfahrens unter Aufrechterhaltung einer Temperatur umfasst, und zwar in (1) einem halbkugelförmigen Raum des 0,5-fachen Ansammlungsabstands d um eine Düsenspitze zum Ansammlungsabstand d zwischen der Spitze einer Spinndüse und einer Sammelfläche von gesponnenen Fasern und/oder (2) einem Punkt von 1 cm auf einer Geraden von der Sammelfläche zum Ansammlungsabstand d zwischen der Spitze der Spinndüse und der Sammelfläche von gesponnenen Fasern bei einer Temperatur, die um 15 °C bis 60 °C über der Glasübergangstemperatur liegt.

## Revendications

1. Étoffe non tissée, comprenant des fibres contenant un polymère ayant une température de transition vitreuse supérieure ou égale à 50 °C comme composant principal, ayant une résistance verticale supérieure ou égale à 1 N/5 cm pour 1 g/m², et satisfaisant les conditions (1) et (2) suivantes : (1) une masse volumique de 0,1 à 0,4 g/cm³ ; et (2) une proportion de parties avec une masse volumique dépassant 0,4 g/cm³ inférieure ou égale à 3 % dans une section transversale dans une direction d'épaisseur,
dans laquelle la résistance verticale est mesurée comme suit : l'étoffe non tissée est coupée en un morceau d'une largeur de 5 cm, et le morceau est étiré à une vitesse de traction de 10 cm/min en utilisant un autographe fabriqué par Shimadzu Corporation conformément à la norme JIS L 1906, et une valeur de charge à un instant de rupture est définie comme la résistance verticale, et
dans laquelle la proportion de parties avec une masse volumique dépassant 0,4 g/cm³ est mesurée comme suit : à l'aide d'un microscope électronique à balayage, une photographie agrandie 100 fois d'une section transversale dans une direction d'épaisseur de l'étoffe non tissée est prise, une ligne droite de 10 mm de la photographie est observée dans une direction de largeur par inspection visuelle, une longueur occupée par des parties avec une masse volumique dépassant 0,4 g/cm³ est mesurée dans cette ligne droite, et la proportion est déterminée par l'équation suivante : $proportion \left(%\right) de parties avec une masse volumique dépassant 0,4 g / {cm}^{3} = longueur de parties avec une masse volumique dépassant 0,4 g / {cm}^{3} \left(mm\right) / 10 \left(mm\right) \times 100 ,$ avec l'observation de la photographie, il est déterminé si la masse volumique dépasse ou non 0,4 g/cm³ en utilisant une fonction de mesure de distance entre deux points rattachés au MEB, et en examinant la longueur des parties avec une masse volumique dépassant 0,4 g/cm³.

2. Étoffe non tissée selon la revendication 1, dans laquelle un taux de fusion de fibres dans une section transversale dans une direction d'épaisseur est supérieur ou égal à 15 %, et une aire moyenne de parties où des fibres sont fusionnées est inférieure ou égale à 70 µm²,
dans laquelle le taux de fusion de fibre est mesuré comme suit : à l'aide d'un microscope électronique à balayage, une photographie agrandie 1 000 fois d'une section transversale dans une direction d'épaisseur de l'étoffe non tissée est prise, et à partir de la photographie, une proportion d'un nombre des sections transversales où deux fibres ou plus sont fusionnées les unes aux autres par rapport à un nombre total des sections transversales de fibre trouvées dans chaque région est déterminée par inspection visuelle et exprimée sous forme de pourcentage sur la base de l'équation suivante : $taux de fusion de fibres ⁢ % = \left(le nombre des sections transversales où deux fibres ou plus sont fusionnées\right) / \left(le nombre total des sections transversales de fibre\right) \times 100 ,$ à condition que le nombre des fibres dont les sections transversales sont vues soit compté dans chaque photographie, et dans un cas où le nombre des sections transversales de fibre est inférieur ou égal à 100, des photographies à observer sont ajoutées de sorte que le nombre total des sections transversales de fibre dépasse 100, et
dans laquelle l'aire moyenne de parties où des fibres sont fusionnées est mesurée comme suit : à l'aide d'un microscope électronique à balayage, une photographie agrandie 1 000 fois d'une section transversale dans une direction d'épaisseur de l'étoffe non tissée est prise, à partir de cette photographie, une aire des parties où des fibres sont fusionnées est calculée, et est divisée par un nombre des parties où des fibres sont fusionnées pour obtenir la valeur moyenne.

3. Étoffe non tissée selon la revendication 1, dans laquelle un diamètre moyen de fibre est de 1 à 10 µm.

4. Étoffe non tissée selon la revendication 1, dans laquelle des fibres à base de polyétherimide amorphe sont contenues.

5. Procédé de production de l'étoffe non tissée selon l'une quelconque des revendications 1 à 4, comprenant la réalisation d'un procédé de fusion-soufflage tout en maintenant une température dans au moins l'un (1) d'un espace hémisphérique de 0,5 x la distance de collecte d autour d'un embout de filière par rapport à la distance de collecte d entre l'embout d'une filière et une surface de collecte de fibres filées, et (2) d'un point de 1 cm depuis la surface de collecte sur une ligne droite par rapport à la distance de collecte d entre l'embout de la filière et la surface de collecte de fibres filées à une température supérieure à la température de transition vitreuse de plus de 15 °C à 60 °C.
